

# United States Patent Office

2,830,021

Patented Apr. 8, 1958

1

2,830,021

## LUBRICANT CONTAINING AN ALIPHATIC AMINE SALT OF MONOALKYL ESTER OF A DIMERIC ACID

Herschel G. Smith, Wallingford, and Troy L. Cantrell, 5 Lansdowne, Pa., assignors to Gulf Oil Corporation, Pittsburgh, Pa., a corporation of Pennsylvania

No Drawing. Application December 28, 1953  
Serial No. 400,748

10 Claims. (Cl. 252—34)

This invention relates to chemical compounds and mineral oil compositions containing the same. More particularly, the invention relates to aliphatic amine salts of monoalkyl esters of dimers of dienoic and trienoic fatty acids. The compounds of this invention have been found to be unusually effective corrosion inhibitors, and they may be advantageously employed as such in mineral oil compositions.

As is well known in the art, "straight" or "uncompounded" mineral oils are often deficient in one or more respects for the particular use to which they are put. For example, a high resistance to rust or corrosion is important for fuels or lubricants which contact metal surfaces in the presence of water. Fuels or lubricants for internal combustion engines and for gas or steam turbines are examples of materials which may desirably have incorporated therein additives or improvement agents which impart corrosion inhibiting properties thereto.

Failure to provide sufficient resistance to rust or corrosion by a particular mineral oil, fuel or lubricant may result in extensive wear or damage to costly, finely-machined moving parts. The damaging effect of rust or corrosion is not necessarily limited to moving parts, since rust particles may flake off and form deposits elsewhere, thereby causing clogging of conduits, valves, filters, screens, etc. To overcome this and other deficiencies of uncompounded mineral oils, various agents known as "addition agents," "additives" or "improvement agents" are commonly incorporated in the particular mineral oil to be used.

The compounds of the present invention form extraordinarily effective corrosion inhibitors which may be used as improvement agents or additives for mineral oils and particularly for lubricating oils such as turbine oils which are required to function in the presence of water. These compounds include the class of amine salts of aliphatic amines having at least one N-substituent containing from 6 to 26 carbon atoms and monoalkyl esters of dimeric acids, these acids being derived from unsaturated fatty acids containing from 6 to 22 carbon atoms and having from 2 to 3 ethylenic linkages per molecule. The invention also includes methods of making the foregoing compounds and in addition includes mineral oil compositions containing compounds of the above-identified class.

The compounds of the present invention may in general be represented by the generic formula:



where



2

is the acyl residue of a dimerized di- or trienoic fatty acid, where  $n$  is an integer of from 10 to 42, where  $x$  is an even integer of from 6 to 10, where  $R_1$  is an aliphatic radical containing from 6 to 26 carbon atoms,  $R_2$  and  $R_3$  are hydrogen or radicals of the same kind as  $R_1$ , and where  $R_4$  is an alkyl group.

The compounds of this invention are prepared by first forming a monoalkyl ester reaction product by partial esterification of a dimerized unsaturated fatty acid of the class indicated with the desired saturated aliphatic, primary, monohydric alcohol. An amine salt of the resulting monoalkyl ester reaction product is formed by neutralizing the monoalkyl ester with the desired aliphatic amine. The partial esterification is effected in conventional manner and under conventional conditions by reacting equimolar proportions of alcohol and dimerized acid. While esterification may proceed slowly at room temperature, the reaction is normally advantageously accelerated by heating the reactants, usually with refluxing, and/or by the use of conventional esterification catalysts such as hydrogen chloride, sulfuric acid, or an aromatic sulfonic acid, such as p-toluenesulfonic acid. The reaction may be driven to substantial completion by removing one of the products of reaction. The use of a monohydric alcohol having a boiling point above that of water is advantageous, since this expedient lends itself to completion of the reaction by removal of the water of esterification through simple distillation. Removal of the water of esterification may be facilitated by mechanical agitation or by bubbling an inert gas, e. g., nitrogen, through the reaction mixture.

The final amine salt reaction product is formed by neutralization or substantial neutralization of the monoalkyl ester with approximately equimolar proportions of the desired amine. In practice, it has been found convenient simply to add sufficient amine to raise the pH of the reaction product to between about 6.5 and about 7.5. The neutralization of the monoalkyl ester of the dimer acid takes place spontaneously at room temperature with the evolution of heat in the instance of primary amines. However, addition of heat is normally required to accelerate the reaction in the instance of secondary or tertiary amines. Care should be exercised, when the neutralization is effected with primary or secondary amines, to prevent the temperature of the reaction mixture from rising above the boiling point of water, in order to avoid amide formation.

The dimerized acids referred to above are dimers, i. e., bimolecular addition products of conjugated or unconjugated dienoic to trienoic fatty acids having from 6 to 22 carbon atoms before dimerization. Dimeric acids derived from dienoic and trienoic fatty acids are well-known and can be prepared by conventional methods which form no part of this invention.

More particularly, dimerized acids capable of forming the compounds of this invention are prepared from di- or trienoic fatty acids having the generic formula  $C_nH_{2n-x}COOH$ , where  $n$  is an integer of from 5 to 21 and  $x$  is 3 or 5. As will be evident, such monomeric acids contain from 6 to 22 carbon atoms and may contain 2 or 3 ethylenic linkages as the ratio of carbon to hydrogen increases, i. e., as  $x$  increases from 3 to 5. Dimerized acids corresponding to the addition products of the foregoing acids therefore may be defined by the generic formula:



where  $n$  is an integer of from 10 to 42 and where  $x$  is an even integer of from 6 to 10. These dimeric acids are therefore dibasic or dicarboxylic acids having from 12 to 44 carbon atoms.

Representative members of the class of dimerized acids capable of forming the compounds of this invention are dimers of dienoic acids such as sorbic (hexadienoic), linoleic (octadecadienoic), humoceric (nonadecadienoic) and eicosinic (eicosadienoic) acids. Dimers of trienoic acids, for example, linolenic and eleostearic (octadecatrienoic) acids also may be used.

It is not necessary that both of the unsaturated fatty acid molecules of the bimolecular addition product be identical. Dimers of mixed composition such as those obtained by dimerizing mixed dienoic, mixed trienoic or mixed dienoic and trienoic acids such as may be derived from certain naturally occurring drying oils are quite satisfactory.

Dienoic and trienoic acids having 18 carbon atoms, especially those having conjugated olefinic linkages, are preferred for reasons of economy of procurement, ease of reaction and the general excellence of the additives prepared therefrom.

As indicated, alcohols capable of forming the above-mentioned monoalkyl esters are the saturated aliphatic, primary, monohydric alcohols, and especially those of lower molecular weight, of which ethyl, hexyl and octyl alcohols are representative. The use of higher alcohols is included by the invention, but such alcohols produce no additional advantage other than a slight increase in the oil-solubility limit of the final reaction product. The alcohols included by the invention may be either straight- or branched-chain. Lower monohydric alcohols having a boiling point above that of water, e. g., butyl, amyl or octyl, are especially suitable, since these alcohols permit the esterification reaction to be carried to completion by distillation of the water formed during the reaction, and also since the oil-solubility of these alcohols render it possible to carry out both the esterification reaction and the neutralization reaction in a mineral oil solution. Such procedure is often advantageous, since it avoids localized overheating of the reactants, and since the product resulting from this procedure is in the form of a mineral oil concentrate containing a relatively high proportion, i. e., up to the solubility limit, of the additive composition. Such mineral oil concentrates of the additives are desirable, since solution of the additive in the ultimate carrier is often greatly facilitated thereby.

Aliphatic amines included for use in the invention are primary, secondary and tertiary amines containing at least one aliphatic N-substituent having from 6 to 26 carbon atoms. The aliphatic N-substituent of the amines may be saturated or unsaturated, straight- or branched-chain, and substituted with groups which do not adversely affect the oil-solubility of the final product. These amines may in general be characterized by the general formula:



where  $R_1$ ,  $R_2$  and  $R_3$  are as defined above.

Illustrative of primary saturated aliphatic amines included in the scope of the invention are the straight- or branched-chain alkyl amines such as hexylamine, hexadecylamine and hexacosylamine. The corresponding unsaturated amines such as hexenyl, hexadecenyl and hexacosenyl amines are representative of suitable unsaturated amines. Secondary and tertiary amines corresponding to the foregoing classes of primary amines may also be used and include not only amines having identical substituents such as dihexylamine, dicyclohexylamine and tridecylamine, but also those having dissimilar substituents such as N,N-hexyl,octadecenylamine.

Preferred amines are the so-called "fatty" amines, i. e., primary alkyl amines containing from 8 to 18 carbon

atoms. Commercial mixtures of fatty amines such as those derived by conventional methods from naturally occurring substances such as coconut oil (cocoamine), palm oil and animal fats or the like are highly suitable.

Representative examples of the herein disclosed class of additive compounds are the octyl, lauryl, octadecyl, octadecenyl, cyclohexyl and dicyclohexyl amine salts of ethyl, butyl, amyl, and octyl dilinoleates and dilinolenates. Examples of the herein disclosed class of com-

The preparation of the herein disclosed class of compounds can be further illustrated by reference to the following specific examples.

### EXAMPLE I

15 Eighty-eight parts by weight of amyl alcohol were admixed with 564 parts by weight of dimerized linoleic acid, and the mixture was heated, trapping off 18 parts by weight of water, over a period of about 4 hours to a maximum temperature for the reaction mixture of 550° F.

The dimerized linoleic acid referred to was a commercial dimeric polymer, manufactured by Emery Industries, Inc., of Cincinnati, Ohio, consisting essentially of dilinoleic acid:



The commercial dimer acid had the following physical properties:

|    |                             |                                  |
|----|-----------------------------|----------------------------------|
| 35 | Physical state              | Straw-colored,<br>viscous liquid |
|    | Molecular weight (approx.)  | 564.                             |
|    | Gravity: °API               | 13.0.                            |
|    | Viscosity, SUV 200° F.      | 597.                             |
| 40 | Flash, OC: °F               | 510.                             |
|    | Fire, OC: °F                | 575.                             |
|    | Color, NPA                  | +10.                             |
|    | Iodine No., Mod. Hanus      | 83.3.                            |
|    | Saponification No           | 186.                             |
|    | Neutralization No           | 182.                             |
| 45 | Dimer content (approx.)     | 85%.                             |
|    | Trimer and higher (approx.) | 12%.                             |
|    | Monomer (approx.)           | 3%.                              |

The reaction product of the above-described esterification reaction, consisting essentially of the monoamyl esters of dilinoleic acid, was cooled to room temperature, and approximately 133 grams of "Armeen 8D" were added. Armeen 8D is a commercial mixture of primary amines, manufactured by Armour & Company of Chicago, Illinois, containing predominantly octylamine together with minor proportions of hexyl and decyl amines and having a mol combining weight of 133 and a melting point of  $-13^{\circ}\text{C}$ . The final reaction product, consisting essentially of the octyl, hexyl and decyl amine salts of monoamyl dilinoleates, was a deep red-colored, viscous liquid having the following properties:

|    |                                    |      |
|----|------------------------------------|------|
| 65 | Gravity: °API                      | 19.1 |
|    | Viscosity, SUV: Sec. 210° F        | 436  |
|    | pH Value, glass-calomel electrodes | 7.5  |
|    | Color ASTM union                   | 7.5  |

Elemental analysis of the reaction product gave the following results:

|                                        |      |
|----------------------------------------|------|
| 70 Analysis, ultimate, percent by wt.: |      |
| Sulfur                                 | 0.1  |
| Hydrogen                               | 12.2 |
| Carbon                                 | 78.2 |
| Oxygen                                 | 7.7  |
| Nitrogen                               | 1.8  |

**5**  
**EXAMPLE II**

To approximately 564 parts by weight of the dimerized linoleic acid of Example I were added 88 parts by weight of amyl alcohol. The mixture was heated under reflux over a period of 4 hours, and 18 parts by weight of water were trapped off the maximum reaction mixture temperature reached being 550° F. The monoamyl ester reaction product was cooled to room temperature and one mol of Armeen CD was added and the mixture stirred. The neutralization reaction proceeded spontaneously with the evolution of heat. "Armeen CD" is a commercial mixture of primary amines, also manufactured by Armour & Company, and derived in known manner from coconut oil. Armeen CD contains a predominant proportion of dodecylamine together with lesser proportions of octyl, decyl, teteradecyl, hexadecyl, octadecyl and octadecenyl amines, has a mol combining weight of 206, and has an approximate melting point of 21° C.

The final product of the foregoing reaction contained predominantly the cocamine salts of monoamyl dilinoleates and was a deep red-colored, viscous liquid having the following properties:

|                                    |      |
|------------------------------------|------|
| Gravity: °API                      | 20.4 |
| Viscosity, S.U.V.: Sec. 210° F.    | 400  |
| pH value, glass-calomel electrodes | 7.5  |
| Color, ASTM union                  | 7.5  |

Elemental analysis of the reaction product gave the following results:

|                                     |      |
|-------------------------------------|------|
| Analysis, ultimate, percent by wt.: |      |
| Sulfur                              | 0.1  |
| Hydrogen                            | 12.4 |
| Carbon                              | 78.3 |
| Oxygen                              | 7.5  |
| Nitrogen                            | 1.7  |

Amine salts of other monoalkyl esters of dimer acids may be obtained in substantially identical fashion by the use of other of the disclosed dimerized fatty acids, alcohols and amines.

The reaction products resulting from the above-described procedures, either alone or in the form of a mineral oil concentrate, may be incorporated in the desired vehicle. Where the vehicle is a mineral lubricating oil, e. g., a turbine oil, the reaction products are employed in a minor proportion sufficient to confer corrosion inhibiting properties upon the latter. Normally from about 0.1 to about 1.0 percent of the additive by weight of the composition is sufficient for this purpose, although greater proportions, i. e., up to 2 or 3 percent by weight, are sometimes desirable and can be used. Examples of various mineral oils which can be benefited by the additives of this invention are gasoline, kerosene, diesel fuel, furnace oil, motor oils, lubricating greases and turbine oils. The invention further includes mineral oil compositions where the solvent constituent is not employed as a fuel or a lubricant but merely as a solvent vehicle. Exemplary of this type of composition are light naphtha and similar solvents containing the novel compounds of this invention. In such instances the compositions find use in the coating art, whereby metallic articles subject to rust or corrosion are brushed, dipped or sprayed with a composition comprising the solvent vehicle and the additive. Subsequent evaporation of the solvent leaves an adherent corrosion-resisting coating of the additive on the article.

As indicated above, the herein disclosed compounds are highly effective corrosion inhibitors. This property of the compounds of this invention has been demonstrated by subjecting lubricating oil compositions containing small concentrations of these additives to the standard, accelerated corrosion tests ASTM D665-47T, procedures A and B. These tests are described in detail in the ASTM Standards of Petroleum Products and Lubri-

cants, November 1948. Very briefly, procedure A of this test involves immersion of a standard steel test rod in an agitated mixture of distilled water and the test oil maintained at a temperature of 140° F. for 48 hours. Procedure B is carried out in substantially identical fashion except that a standard, synthetic sea water solution is substituted for the distilled water of procedure A. The corrosion inhibiting properties of the oil are determined by examination of the steel rod for rust or corrosion at the conclusion of the test.

The following specific examples are illustrative of the results obtainable by the compounds of this invention.

**EXAMPLE III**

To a highly refined, highly paraffinic turbine oil base having an API gravity of between 30.5° and 32.5° and a viscosity of about 150 SUS at 100° F., and which had been inhibited against oxidation, was added 0.15 percent by weight of the composition of the additive prepared according to Example I. Samples of the improved turbine oil and unimproved turbine oil base were tested according to procedures A and B, ASTM D665-47T. The results of these tests are presented in the table below:

*Table A*

|                                                                                                                           | Base Oil              | Base Oil plus 0.15% by wt. Product of Ex. I |
|---------------------------------------------------------------------------------------------------------------------------|-----------------------|---------------------------------------------|
| Corrosion Test ASTM D665-47T, Procedure A, Distilled Water, 48 Hrs.:<br>Steel Rod, Appearance                             | rusted...<br>100..... | bright.<br>0.....                           |
| Corrosion Test ASTM D665-47T, Procedure B, Synthetic Sea Water, 48 Hrs.:<br>Steel Rod, Appearance<br>Area Rusted, percent | rusted...<br>100..... | bright.<br>0.....                           |

**EXAMPLE IV**

To a turbine oil base of the same type as that described in Example III was added 0.15 percent by weight of the additive prepared according to Example II. The improved turbine oil and the unimproved turbine oil base were each tested according to procedures A and B of ASTM D665-47T. The results of these tests are presented in the following table:

*Table B*

|                                                                                                                           | Base Oil              | Base Oil plus 0.15% by wt. Product of Ex. II |
|---------------------------------------------------------------------------------------------------------------------------|-----------------------|----------------------------------------------|
| Corrosion Test ASTM D665-47T, Procedure A, Distilled Water, 48 Hrs.:<br>Steel Rod, Appearance<br>Area Rusted, percent     | rusted...<br>100..... | bright.<br>0.....                            |
| Corrosion Test ASTM D665-47T, Procedure B, Synthetic Sea Water, 48 Hrs.:<br>Steel Rod, Appearance<br>Area Rusted, percent | rusted...<br>100..... | bright.<br>0.....                            |

The herein disclosed derivatives of dimerized unsaturated fatty acids are markedly more effective as corrosion inhibitors than the parent dimer acid itself, as illustrated by a comparison of the foregoing results with those presented in the following example.

**EXAMPLE V**

To separate samples of a turbine oil base of the same type described in Example III were added respectively 0.2 percent and 0.3 percent by weight of the dimerized linoleic acid described in Example I. These samples were tested according to procedures A and B of ASTM D665-47T. The results of these tests are shown below,

7  
Table C

|                                                                                                     | Base Oil<br>plus 0.2%<br>by wt. Di-<br>merized<br>Linoleic<br>Acid | Base Oil<br>plus 0.3%<br>by wt. Di-<br>merized<br>Linoleic<br>Acid |
|-----------------------------------------------------------------------------------------------------|--------------------------------------------------------------------|--------------------------------------------------------------------|
| Corrosion Test ASTM D665-47T, Procedure A, Distilled Water, 48 Hrs.: Steel Rod, Appearance.....     | rusted.....<br>70.....                                             | rusted.....<br>70.....                                             |
| Area Rusted, percent.....                                                                           |                                                                    |                                                                    |
| Corrosion Test ASTM D665-47T, Procedure B, Synthetic Sea Water, 48 Hrs.: Steel Rod, Appearance..... | rusted.....<br>100.....                                            | rusted.....<br>100.....                                            |
| Area Rusted, percent.....                                                                           |                                                                    |                                                                    |

Examination of Tables A and B indicates that low concentrations of the compounds of this invention impart extremely high corrosion inhibiting properties to oils, even under the extremely severe conditions of the ASTM procedure B accelerated corrosion test.

Comparison of the results given in Tables A, B and C shows that our amine salt-monoalkyl ester derivatives produce as much as 100 percent improvement in results even when used in concentrations as little as one-half as much as the parent dimer acid. The herein disclosed compounds also impart more persistent corrosion inhibiting properties to mineral oils than do the parent dimeric acids.

It is to be understood that the improved mineral oil compositions of this invention can be additionally improved by incorporation therein of other known additives in order to confer thereon other desirable properties, such as increased resistance to oxidation, increased stability, etc. Thus, there can be added viscosity index improvers, thickeners, bearing corrosion inhibitors, anti-oxidants, extreme pressure agents, foam inhibitors, dyes, sludge inhibitors, detergents, etc.

The additive compounds included by the invention also find utility as corrosion-inhibiting additives for various paints, varnishes, automobile undercoatings and the like. In the use of the agents of this invention in the above-described coating compositions, it may be desirable to employ these agents in substantially greater concentrations than are normally utilized in fuels and lubricants.

It will be understood by those skilled in the art that numerous modifications may be resorted to without departing from the spirit of the invention or scope of the appended claims.

We claim:

1. An amine salt of (1) an aliphatic amine having at least one N— substituent containing from 6 to 26 carbon atoms and (2) a monoalkyl ester of a dimeric acid, said dimeric acid being derived from an unsaturated fatty

acid containing from 6 to 22 carbon atoms and having from 2 to 3 ethylenic linkages per molecule.

2. The compound of claim 1 wherein the unsaturated fatty acid contains 18 carbon atoms.

3. An amine salt of a primary alkyl amine containing from 8 to 18 carbon atoms and a monoamyl dilinoleate.

4. A method of preparing an amine salt of a mono-alkyl ester of a dimerized unsaturated fatty acid, comprising forming a monoalkyl ester by reacting substantially equimolar proportions of a saturated aliphatic primary monohydric alcohol and a dimeric acid derived from an unsaturated fatty acid containing from 6 to 22 carbon atoms and having from 2 to 3 ethylenic linkages per molecule, and forming an amine salt of said mono-alkyl ester by neutralizing the same with an aliphatic amine having at least one N— substituent containing from 6 to 26 carbon atoms.

5. A mineral oil composition comprising a major amount of a mineral oil and a minor amount, sufficient to impart corrosion inhibiting properties to the composition, of an amine salt of (1) an aliphatic amine having at least one N— substituent containing from 6 to 26 carbon atoms and (2) a monoalkyl ester of a dimeric acid, said dimeric acid being derived from an unsaturated fatty acid containing from 6 to 22 carbon atoms and having from 2 to 3 ethylenic linkages per molecule.

6. The composition of claim 5 wherein the mineral oil is a lubricating oil.

7. The composition of claim 5 wherein the mineral oil is a turbine oil.

8. The composition of claim 5 wherein the unsaturated fatty acid contains 18 carbon atoms.

9. A mineral oil composition comprising a major amount of a mineral oil and a minor amount, sufficient to impart corrosion inhibiting properties to the composition, of an amine salt of a primary alkyl amine containing from 8 to 18 carbon atoms and a monoamyl dilinoleate.

10. The composition of claim 9 wherein the amine salt is present in concentrations of from about 0.01 to about 1.0 percent by weight of the composition.

#### References Cited in the file of this patent

#### UNITED STATES PATENTS

|           |              |                |
|-----------|--------------|----------------|
| 2,162,454 | Guthmann     | June 13, 1939  |
| 2,366,013 | Duncan       | Dec. 26, 1944  |
| 2,399,510 | Rocchini     | Apr. 30, 1946  |
| 2,564,422 | Barnum       | Aug. 14, 1951  |
| 2,587,546 | Matuszak     | Feb. 26, 1952  |
| 2,631,979 | McDermott    | Mar. 17, 1953  |
| 2,689,828 | Smith et al. | Sept. 21, 1954 |